

## UNITED STATES PATENT OFFICE.

BARTHOLOMÄUS VOSSEN, OF HOCHST-ON-THE-MAIN, GERMANY, ASSIGNOR TO GRAS-SELLI DYESTUFF CORPORATION, OF NEW YORK, N. Y., A CORPORATION OF DELAWARE.

## PROCESS OF DYEING LEATHER WITH ACID AZO DYESTUFFS.

No Drawing. Application filed January 23, 1926, Serial No. 83,389, and in Germany February 3, 1925.

I have found that deep and full brown dyeings can be produced on leather tanned by any method and this with such a depth of shade as could hitherto not at all be obtained 5 in the art of dyeing leather by means of acid azo dyestuffs or only by means of mixtures of various dyestuffs of this kind, if there are used dyestuffs formed according to the following scheme:



In this scheme the term "amine" (I and IV) comprises:

15      All diazotizable aromatic amines, amino-hydroxy and amino-azo compounds and also their substitution products including the sulfonic acids and carboxylic acids, for instance aniline, p-nitraniline, aminoazobenzene, 20 2-chlor-6-toluidine-4-sulfonic acid, p-nitro-o-aminophenol, picramic acid, naphthionic acid, or the like;

The term "non-sulfonated resorcinol" (II) comprises:

25      Resorcinol and its substitution products including the carboxylic acids with the exception of the respective sulfonic acids, for instance resorcinol, chlorresorcinol, 1,3,4-resorcylic acid or the like;

30      The acids mentioned under III comprise:

Aminonaphtholmono- or disulfonic acids as well as naphthyl-aminemono- or disulfonic acid, for instance 1-amino-8-hydroxynaphthalene-3,6-disulfonic acid (H acid), 1-amino-8-hydroxynaphthalene-4,6-disulfonic acid (K acid), 1-amino-8-hydroxynaphthalene-4-sulfonic acid, and the technical mixture of 1-naphthylamine-6-sulfonic acid and 1-naphthylamine-7-sulfonic acid; and the arrow points from the amino compound which

35      is diazotized to the compound with which the diazotized amino compound is coupled.

40      Some of the dyestuffs of the aforementioned type are already known, but they were hitherto only described as being suitable for use as acid or chrome mordant dyestuffs for wool. They were, however, not adopted to a great extent, probably owing to their unsatisfactory levelling power and the insufficient fastness of the dyeings obtained therewith on wool.

45      It could not at all be foreseen that the dyestuffs prepared according to the foregoing scheme, which are almost of no value for dye- 55

ing wool, are eminently suitable for dyeing leather. The dyestuffs belonging to this class are particularly distinguished by the beautiful tints they give on leather and they are therefore of great value in the art of leather dyeing. Moreover they enable the 60 leather-dyers to obtain deep and full brown tints on leather by means of a single dyestuff and thus to abandon the use of dyestuff mixtures hitherto required for obtaining the said tints, which mixtures were 65 apt to cause difficulties in the dyeing process. The dyestuffs belonging to the said type also possess excellent covering and levelling properties so much so that not only the grain of the leather but also the defective spots on it 70 are dyed even tints of even depth. Such even dyeings on leather could not be obtained by the hitherto used dyestuff mixtures, because the various components of such mixtures are apt to give on the defective spots a 75 tint which differs from that of the grain.

The fastness of the dyeings obtainable on leather by the dyestuffs in question entirely satisfy the requirements to be made in regard to dyeings on leather. 80

The method of dyeing with the dyestuff of the above defined composition is the same as that generally used in dyeing with acid azo dyestuffs.

The following example will illustrate my 85 invention:

300 kg. of chrome leather, which has been well freed from acid, is soaked in a rotating cask with 150 litres of hot water of 60° C. and there is then added a solution of 1,5 kg. of the 90 dyestuff: picramic acid → 1-amino-8-hydroxynaphthalene-3,6-disulfonic acid → resorcinol → p-nitraniline in 50 litres of hot water by slowly introducing this solution through the hollow axis of the cask. After the said operation has been continued for 10 minutes, there are slowly added 200 cc. of formic acid of 85% strength diluted with 2 litres of water, and the operation is continued for another 20 minutes. Thereupon there is added a fat as 95 usual.

In the same manner may be dyed bark-tanned sheepskin-leather and kid-leather with the only exception that in these cases the addition of a fat may be omitted.

100 Instead of the dyestuff indicated in the foregoing example there may be used in the same manner for dyeing the leather the fol-

lowing dyestuffs or dyestuffs of similar composition viz:—

2-amino-1-methylbenzene-5-sulfonic acid→  
1 - amino - 8 - hydroxynaphthalene - 3.6 - di-  
5 sulfonic acid→resorcinol←p-nitraniline

sulfanilic acid→1-amino-8-hydroxynaphthalene-3.6-disulfonic acid→resorcinol←p-nitraniline

10 naphthionic acid→1 - amino - 8 - hydroxy-  
naphthalene - 3.6-disulfonic acid→resorcinol←p-nitraniline

15 sulfanilic acid→technical mixture of 1-naphthylamine-6-sulfonic acid and 1-naphthylamine-7-sulfonic acid→resorcinol←4-nitro-2-amino-1-phenol

4-nitro-2-amino-1-phenol→technical mixture as aforesaid→resorcinol←naphthionic acid

20 picramic acid→technical mixture as aforesaid→resorcinol←picramic acid.

I claim:

25 1. The process of dyeing leather in full brown shades of even depth with acid azo dyestuffs, which comprises using for the dyeing process dyestuffs formed according to the scheme:



30 wherein I and IV each stand for a diazotizable aromatic amine, aminohydroxy- or amino-azo compound or a substitution product thereof, II stands for non-sulfonated resorcinol or a substitution product thereof, and III stands for an aminonaphthol mono- or disulfonic acid.

2. The process of dyeing leather in full brown shades of even depth with acid azo dyestuffs, which comprises using for the dyeing process dyestuffs formed according to the scheme:



40 45 wherein R in I stands for an aromatic nucleus which may contain an  $\text{NO}_2$  group, II stands for non-sulfonated resorcinol or a substitution product thereof, III stands for an aminonaphthol mono- or disulfonic acid, IV stands for a diazotizable aromatic amine, aminohydroxy- or amino-azo compound or a substitution product thereof.

50 55 3. The process of dyeing leather in full brown shades of even depth with acid azo dyestuffs, which comprises using for the dyeing process dyestuffs formed according to the scheme:



60 wherein IV stands for a diazotizable aromatic amine, aminohydroxy- or amino-azo compound or a substitution product thereof.

65 70 4. The process of dyeing leather in full brown shades of even depth with acid azo dyestuffs, which comprises using for the dyeing process a dyestuff formed according to the scheme:



In testimony whereof, I affix my signature.

BARTHOLOMÄUS VOSSEN.